

## UNITED STATES PATENT OFFICE

2,610,122

SILVER HALIDE DEVELOPER CONTAINING  
2(β-HYDROXYETHYL)AMINOPHENOL AND  
p-HYDROXYPHENYLAMINO ACETIC ACID

David Hugh Oakley John, Hornchurch, and  
George Terence James Field, London, England,  
assignors to May & Baker Limited, Dagenham,  
England, a British company

No Drawing. Application May 12, 1950, Serial No.  
161,734. In Great Britain July 31, 1948

9 Claims. (Cl. 95—88)

1

This invention relates to photographic developers and particularly to fine grain photographic developers.

In British Patent No. 295,939, 2(β-hydroxyethyl)aminophenol is suggested as a photographic developer and developer formulae have been produced based on the use of this compound which give fine grain results. A suitable formula using this compound is as follows:

## DEVELOPER A

|                                       | Grams |
|---------------------------------------|-------|
| 2(β-hydroxyethyl)aminophenol sulphate | 6     |
| Sodium sulphite anhydrous             | 100   |
| Sodium carbonate anhydrous            | 11.5  |
| Sodium hexametaphosphate              | 1.7   |
| Potassium bromide                     | 0.6   |
| Water to make 1 litre.                |       |

The developer so constituted gives a very fine grain but it has the disadvantage that it develops rather slowly. There is set out below a comparison between this developer and other standard developers in which this point is brought out:

| Developer   | Emul-<br>sion<br>Speed | Gramu-<br>larity<br>Index | Fog<br>Level | Develop-<br>ment<br>Time in<br>Minutes |
|-------------|------------------------|---------------------------|--------------|----------------------------------------|
| Developer A | 91                     | 110                       | 0.04         | 18                                     |
| Developer B | 33                     | 100                       | 0.04         | 40                                     |
| Developer C | 100                    | 175                       | 0.09         | 7                                      |
| Developer D | 100                    | 240                       | 0.11         | 5                                      |

In this table the terms have the following meanings:

*Emulsion speed.*—Developer C is taken as giving a speed of 100 and all other speed data are expressed as a percentage of this maximum. The speed estimation is based on the determination of the inertia point and a developer giving a speed of 50 would therefore demand twice the initial exposure to give the result of Developer C.

*Granularity index.*—The granularity given by Developer B is assigned the index 100. All other granularities have been expressed relative to this, the lower the figure the less pronounced is the grain.

*Fog level.*—This term has its usual significance in this field, being the density of the silver image obtained in the area which has not been exposed to light.

*Development time.*—This is the time required in minutes to give a gamma of 1.0, development being effected at 68° F.

The standard developers with which the

2(β-hydroxyethyl)aminophenol developer is compared have the following formulae:

## DEVELOPER B

|                           | Grams |
|---------------------------|-------|
| p-Phenylene diamine base  | 10    |
| Sodium sulphite anhydrous | 90    |
| Water to make 1 litre.    |       |

## DEVELOPER C

|                             | Grams |
|-----------------------------|-------|
| p-Methylaminophenolsulphate | 2     |
| Sodium sulphite anhydrous   | 100   |
| Hydroquinone                | 5     |
| Borax                       | 2     |
| Water to make 1 litre.      |       |

## DEVELOPER D

|                             | Grams |
|-----------------------------|-------|
| p-Methylaminophenolsulphate | 2     |
| Sodium sulphite anhydrous   | 75    |
| Sodium carbonate anhydrous  | 37    |
| Hydroquinone                | 3     |
| Potassium bromide           | 2     |
| Water to make 1 litre.      |       |

It will be seen from the foregoing comparison that the 2(β-hydroxyethyl)aminophenol developer compares very favourably as a fine grain developer, that is to say it gives an emulsion speed closely comparable with those of Developers C and D and yet whereas the granularity indexes of these latter developers are 175 and 240 respectively the granularity index of the 2(β-hydroxyethyl)aminophenol developer is only 110. The fog level obtained with 2(β-hydroxyethyl)aminophenol developer is low and the main criticism of it is that its development time (18 minutes), while much better than Developer B, is nevertheless long compared with that of Developer C.

It is an object of this invention to provide new developer compositions yielding fine grain developer images with much reduced development time. It is a further object of this invention to provide concentrated developer compositions of such a character which merely require dilution with water for use. It is a still further object of this invention to provide such developer compositions in the form of dry powders merely requiring dissolution in water to produce developing solutions. A further object is to provide methods of developing photographic silver halide emulsions whereby fine grain fully developed images may be obtained in a short developing time.

It has now been discovered that the inclusion in a developer based on 2(β-hydroxyethyl) -

aminophenol (usually employed as the sulphate) of a quantity of p-hydroxyphenylamino acetic acid, i. e. photographic glycine, reduces very considerably the development time without having any appreciable effect on any of its other characteristics.

According to the present invention, therefore, a photographic developer for silver halide emulsions comprises 2(β-hydroxyethyl)aminophenol and p-hydroxyphenylamino acetic acid, and more particularly according to the invention the developer comprises these two compounds in aqueous alkaline solution and particularly in association with alkali sulphites, e. g. sodium sulphite, alkali carbonates, e. g. sodium carbonate, and other compounds common to photographic developers. Such other compounds may be, for example, borax, sodium metaborate, tri-sodium phosphate and sodium hexametaphosphate. The potassium and ammonium salts of any of these compounds may, of course, alternately be employed.

The concentration of 2(β-hydroxyethyl) aminophenol (calculated as sulphate) should generally be not less than 4 or more than 8 grams per litre and the proportion of p-hydroxyphenylamino acetic acid may conveniently be from 10 to 30% of the weight of the former compound.

The following is an example of a photographic fine grain developer made in accordance with the present invention:

*Example*

|                                       | Grams |
|---------------------------------------|-------|
| 2(β-hydroxyethyl)aminophenol sulphate | 6     |
| p-Hydroxyphenylamino acetic acid      | 1.13  |
| Sodium sulphite anhydrous             | 100   |
| Sodium carbonate anhydrous            | 11.5  |
| Sodium hexametaphosphate              | 1.7   |
| Water to make 1 litre.                |       |

This developer was compared with Developer A and also with Developer A modified by the omission of the potassium bromide, and gave the following results:

|                                            | Emul-<br>sion<br>Speed | Granu-<br>larity<br>Index | Fog<br>Level | Devel-<br>opment<br>Time in<br>Minutes |
|--------------------------------------------|------------------------|---------------------------|--------------|----------------------------------------|
| Developer A                                | 91                     | 110                       | 0.04         | 18                                     |
| Developer A omitting the potassium bromide | 91                     | 115                       | 0.12         | 16                                     |
| Developer of the Example                   | 90                     | 115                       | 0.11         | 8                                      |

From these results it is clear that the emulsion speed and granularity index given by the three developers is substantially identical. The fog level increase shown by the last two developers is not serious in practice. On the other hand whereas a small decrease in development time can be achieved by omitting the potassium bromide from Developer A, the effect of including p-hydroxyphenylamino acetic acid is to reduce the development time by more than half.

The invention includes the new developers in the form of solutions (ready for use or highly concentrated) and also in the form of dry packed powders.

We claim:

1. A photographic developer for silver halide emulsions which comprises a salt of 2(β-hydroxyethyl)aminophenol, p-hydroxyphenylamino acetic acid and an alkali carbonate in aqueous solution the concentration of 2(β-hydroxyethyl)aminophenol (calculated as sulphate) being be-

tween 4 and 8 grams per litre, and the concentration of p-hydroxyphenylamino acetic acid being from 10-30% of the said concentration of 2(β-hydroxyethyl)aminophenol.

5. A photographic developer for silver halide emulsions which comprises a salt of 2(β-hydroxyethyl)aminophenol, p-hydroxyphenylamino acetic acid, an alkali carbonate and an alkali sulphite in aqueous solution the concentration of 2(β-hydroxyethyl)aminophenol (calculated as sulphate) being between 4 and 8 grams per litre, and the concentration of p-hydroxyphenylamino acetic acid being from 10-30% of the said concentration of 2(β-hydroxyethyl)aminophenol.

10. 3. A photographic developer for silver halide emulsions which comprises a salt of 2(β-hydroxyethyl)aminophenol, p-hydroxyphenylamino acetic acid, an alkali carbonate, an alkali sulphite and sodium hexametaphosphate in aqueous solution the concentration of 2(β-hydroxyethyl)aminophenol (calculated as sulphate) being between 4 and 8 grams per litre, and the concentration of p-hydroxyphenylamino acetic acid being from 10-30% of the said concentration of 2(β-hydroxyethyl)aminophenol.

15. 4. A photographic developer for silver halide emulsions comprising a salt of 2(β-hydroxyethyl)aminophenol and p-hydroxyphenylamino acetic acid in aqueous alkaline solution, the concentration of 2(β-hydroxyethyl)aminophenol (calculated as sulphate) being between 4 and 8 grams per litre, and the concentration of p-hydroxyphenylamino acetic acid being from 10-30% of the said concentration of 2(β-hydroxyethyl)aminophenol.

20. 5. A photographic developer for silver halide emulsions containing the following ingredients in substantially the following proportions:

|                                       | Grams |
|---------------------------------------|-------|
| 2(β-hydroxyethyl)aminophenol sulphate | 6     |
| p-Hydroxyphenylamino acetic acid      | 1.13  |
| Sodium sulphite anhydrous             | 100   |
| Sodium carbonate anhydrous            | 11.5  |
| Sodium hexametaphosphate              | 1.7   |
| Water to make 1 litre.                |       |

40. 6. A dry photographic developer composition for silver halide emulsions comprising a salt of 2(β-hydroxyethyl)aminophenol, p-hydroxyphenylamino acetic acid and an alkali the proportion of p-hydroxyphenylamino acetic acid being 10-30% by weight of the said salt.

45. 7. A dry photographic developer composition for silver halide emulsions comprising a salt of 2(β-hydroxyethyl)aminophenol, p-hydroxyphenylamino acetic acid, an alkali sulphite and an alkali carbonate the proportion of p-hydroxyphenylamino acetic acid being 10-30% by weight of the said salt.

50. 8. Process for the development of a photographic silver halide emulsion which comprises subjecting an exposed photographic element carrying a layer of such emulsion to treatment with a developer comprising a salt of 2(β-hydroxyethyl)aminophenol and p-hydroxyphenylamino acetic acid in aqueous alkaline solution the concentration of 2(β-hydroxyethyl)aminophenol (calculated as sulphate) being between 4 and 8 grams per litre, and the concentration of p-hydroxyphenylamino acetic acid being from 10-30% of the said concentration of 2(β-hydroxyethyl)aminophenol.

55. 9. Process for the development of a photographic silver halide emulsion which comprises

70. 75.

subjecting an exposed photographic element carrying a layer of such emulsion to treatment with a developer comprising a salt of 2(β-hydroxyethyl)aminophenol, p-hydroxyphenylamino acetic acid, an alkali carbonate and an alkali sulphite in aqueous solution the concentration of 2(β-hydroxyethyl)aminophenol (calculated as sulphate) being between 4 and 8 grams per litre, and the concentration of p-hydroxyphenylamino acetic acid being from 10-30% of the said concentration of 2(β-hydroxyethyl)aminophenol.

DAVID HUGH OAKLEY JOHN.

GEORGE TERENCE JAMES FIELD.

#### REFERENCES CITED

The following references are of record in the file of this patent:

#### UNITED STATES PATENTS

| Number    | Name      | Date         |
|-----------|-----------|--------------|
| 1,758,762 | Reddelien | May 13, 1930 |

#### OTHER REFERENCES

10 Henney & Dudley: "Handbook of Photography," McGraw-Hill, New York, 1939, page 335.